

Dec. 24, 1957

P. R. TEMPLIN

2,817,640

WAX COMPOSITION AND FIBROUS MATERIAL COATED THEREWITH

Filed April 12, 1955



INVENTOR.  
PHILIP R. TEMPLIN  
BY

*Donald L. Carson*

HIS ATTORNEY

1

2,817,640

## WAX COMPOSITION AND FIBROUS MATERIAL COATED THEREWITH

Philip R. Templin, Oakmont, Pa., assignor to Gulf Research & Development Company, Pittsburgh, Pa., a corporation of Delaware

Application April 12, 1955, Serial No. 500,827

20 Claims. (Cl. 260—28.5)

This invention relates to an improved wax composition, more particularly to an improved paraffin wax composition having superior heat-sealing properties, and to a fibrous material coated therewith.

The employment of paraffin waxes has undergone a rapid growth in recent years. Thus, large quantities of paraffin wax compositions have found their way into the impregnation and coating of fibrous materials such as paper, fiber board, laminated papers, etc. These compositions have also found wide use in the waterproofing of various textiles and papers and in the formation of protective coatings.

Among the uses for wax compositions has been as bonding agents in the adhesive bonding technologies such as the wrapping paper industry and the coated and laminated paper industry. Examples of these uses can be found in the waxed paper employed in wrapping food such as bread, frozen foods, breakfast foods, etc., paper-board cartons and drums, paper milk containers, bottle cap liner coatings, drinking cups, etc., and the various laminated paper compositions. When applied to these uses, one of the most valuable properties of the wax composition is its sealing strength. Thus, in the case of a wrapping paper, a poor seal requires a costly rewapping of the package at the wrapping machine and, more seriously, can result in broken packages during subsequent handling. Moreover, the formation of a poor seal must be compensated for by expensive reinforcement techniques, such as the use of excessive amounts of paper for a seal overlap and the use of end labels or tabs for reinforcement. The use of these reinforcement techniques has proved costly in terms of time, material, unit production, customer good will, etc. In the case of laminates a wax of low sealing strength effectuates peeling and separation of the laminated layers.

Moreover, wax compositions possessing other properties such as high tensile strength have also found wide use in the packaging industry. Thus, a highly successful use for wax compositions has been in the manufacture of certain types of paper milk containers, e. g., paper containers coated with paraffin wax or paraffin wax compositions. It is desirable that the wax employed for coating these paper containers possess a high tensile strength.

I have found that an improved paraffin wax composition which possesses a very high sealing strength, and also superior tensile strength, can be prepared comprising paraffin wax, a rubbery isobutylene polymer and a long-chain alcohol wax.

My invention is broadly applicable to paraffin waxes in general. By "paraffin wax" I mean to include the hard, crystalline hydrocarbon waxes such as are derived from mineral oils of the mixed base or paraffinic base type, or from shale oils, or the Fischer-Tropsch synthesis of hydrocarbons. The invention is particularly applicable to paraffin waxes having a melting point of about 90° to about 160° F., preferably of about 120° to about 150° F.

By "rubbery isobutylene polymer" I mean to include

2

polymerized isobutylenes such as polyisobutylene and isobutylene copolymer rubbers with at least 75 percent and preferably 95 percent or more by weight of the hydrocarbon polymer derived from isobutylene. The molecular weight of the polyisobutylene is not critical and can be varied over a wide range. While polyisobutylene having a Flory molecular weight as low as about 5,000 can be used, I prefer to employ polyisobutylenes having a Flory molecular weight greater than about 30,000, preferably of about 55,000 to about 1,325,000. As indicated above, the isobutylene copolymer rubbers comprise high molecular weight polymers containing at least 95 percent by weight of the hydrocarbon as isobutylene constituent. The remainder can comprise, for example, an olefinic-type compound such as butene, or a compound having a conjugated system of multiple bonds in which at least one of the multiple bonds is an ethylenic double bond. Examples of the last-mentioned type compound include styrene, acrylonitrile, methacrylonitrile, methacrylic acid, esters of methacrylic acid, butadiene, isoprene and chlorobutadiene. The preferred isobutylene copolymer employed herein contains 97 to 98 percent of isobutylene constituent and 2 to 3 percent of isoprene constituent.

By "Flory molecular weight" I mean the viscosity average molecular weight obtained by the method for determining the molecular weights of polymers devised by Paul J. Flory and Thomas G. Fox, Jr., set forth in the Journal of Polymer Science, volume 5, pages 745-747 (1950). Briefly, this method is based upon a determination of the intrinsic viscosity ( $N_1$ ) of a solution of the polymer in a solvent, such as benzene, at a fixed temperature, such as 24° C. The Flory molecular weight (M), constituting a viscosity average molecular weight, is then determined from the following formula:

$$M^{1/2} = N_1 / (K\alpha^3)$$

where K is a constant, which is  $1.07 \times 10^{-3}$  for polyisobutylene at 24° C., and  $\alpha$  is a linear expansion factor equal to unity at 24° C. for polyisobutylene. The intrinsic viscosity ( $N_1$ ) is the limiting value of the ratio of the specific viscosity ( $N_{sp}$ ) to the concentration of polymer at infinite dilution. The intrinsic viscosity ( $N_1$ ) is determined by plotting the ratio of the specific viscosity ( $N_{sp}$ ) to the concentration of polymer against the concentration of the polymer and extrapolating the resultant plot to zero concentration. The specific viscosity ( $N_{sp}$ ) is equal to the relative viscosity ( $N_r$ ) minus one, i. e.,  $N_{sp} = N_r - 1$ , the relative viscosity ( $N_r$ ) being the ratio of the viscosity of the solution of the polymer to the viscosity of the solvent.

Accordingly, to effect a Flory molecular weight determination, the relative viscosity ( $N_r$ ) is determined for several different concentrations of the polymer in the solvent. From these several relative viscosities ( $N_r$ ), the corresponding specific viscosities ( $N_{sp}$ ) are calculated, as well as the ratios of the calculated specific viscosities ( $N_{sp}$ ) to the corresponding concentrations. The ratios thus obtained are plotted against the corresponding concentrations and the straight line plot is extrapolated to zero concentration, thereby providing the intrinsic viscosity ( $N_1$ ).

Among the long-chain alcohol waxes which can be employed in the preparation of the paraffin wax compositions of this invention are saturated long-chain alcohol waxes, branched and straight chain, having from one to about 50 hydroxyl groups per molecule, preferably from one to about 25 hydroxyl groups per molecule, the structural formula of which can be written as follows:



wherein  $k$  is an integer from about 50 to about 310, preferably about 100 to about 200, and  $m$  is an integer from one to about 50, preferably one to about 25. The location of the hydroxyl groups in the long-chain alcohol waxes employed herein can be varied as desired in the molecule and branching can occur within the limits of the structural formula defined above without adversely affecting the sealing and tensile strength properties thereof when such alcohol waxes are employed in combination with a rubbery isobutylene polymer as additives for paraffin waxes. Any long-chain alcohol wax encompassed by the formula defined above having the required number of hydroxyl groups will improve the sealing and tensile strength of paraffin wax when added thereto in admixture with a rubbery isobutylene polymer. The production of the type of long-chain alcohol waxes suitable for use in admixture with rubbery isobutylene polymers and paraffin waxes in accordance with this invention is shown and described, for example, in U. S. Patent No. 2,504,400 to Erchak, Jr.

As noted, the improved paraffin wax compositions of this invention comprising paraffin wax, a rubbery isobutylene polymer and a long-chain alcohol wax possess a very high sealing strength and superior tensile strength. Unexpectedly, I have found that paraffin wax compositions comprising paraffin wax and a rubbery isobutylene polymer and a long-chain alcohol wax, when employed within limits hereinafter defined, have a higher sealing strength than compositions comprising only paraffin wax and a rubbery isobutylene polymer or paraffin wax and a long-chain alcohol wax.

While my improved paraffin wax compositions can be prepared with a major amount of a paraffin wax and as low as about 0.01 weight percent, based on the final paraffin wax compositions, of combined rubbery isobutylene polymer and long-chain alcohol wax, I prefer to employ the combined rubbery isobutylene polymer and long-chain alcohol wax in amounts in excess thereof. For best results, the combined rubbery isobutylene polymer and long-chain alcohol wax should be present in an amount greater than about 0.1 percent by weight, and can be present in an amount up to about 50 percent by weight but preferably about one to about 10 percent by weight. The ratio of rubbery isobutylene polymer to long-chain alcohol wax present in the final paraffin wax composition is exceedingly important in obtaining a paraffin wax composition having a higher sealing strength than one containing only paraffin wax and a rubbery isobutylene polymer or only paraffin wax and a long-chain alcohol wax. I have found that in such case of the combined total of rubbery isobutylene polymer and long chain alcohol wax, the weight percent of the rubbery isobutylene polymer must be about 92 to about 46 percent, preferably about 86 to about 52 percent, while the weight percent of the long-chain alcohol wax must be about 8 to about 54 percent, preferably about 14 to about 48 percent. As to the tensile strength of the paraffin wax compositions of this invention, however, the tensile strength increases as a straight line function by increased additions of the two, the tensile strength increase thereof being more pronounced as the ratio of long-chain alcohol wax to rubbery isobutylene polymer increases.

In preparing the paraffin wax compositions of this invention any method that will effect mixing of the three components forming a part thereof and assure the obtaining of a homogeneous mixture can be used. Thus, a convenient and effective method of obtaining the paraffin wax mixture is to place the ingredients in a container, heat the contents thereof to a temperature of about 100° C., and thereupon mix the heated contents, using an Eppenbach homomixer, until a homogeneous solution has been obtained. Depending upon the quality and grade of ingredients employed and other factors involved, the length of time necessary for mixing can be as low as about 15 minutes or as much as three to four hours.

The invention can best be illustrated by the following examples:

#### EXAMPLE I

5 Into a container are placed, based upon the weight of the final composition, 95 percent by weight of paraffin wax having a melting point of 133° F., and a combined total of 5 percent by weight of Alcowax 7 (a product of the Semet-Solvay Division of Allied Chemical and Dye Corporation) found upon analysis to possess the following structural formula:  $C_{149}H_{289}OH$  and polyisobutylene having a Flory molecular weight of 84,000. The long-chain alcohol wax and the polyisobutylene are employed in the following ratios: 5:0, 4:1, 3:2, 2.5:2.5, 2:3, 1:4 and 0:5. The ingredients are heated to a temperature of about 100° C. and mixed with an Eppenbach homomixer for about one hour until a homogeneous mixture is obtained.

#### EXAMPLE II

20 Into a container are placed, based upon the weight of the final composition, 95 percent by weight of paraffin wax having a melting point of 133° F., and a combined total of 5 percent by weight of Alcowax M (a product of the Semet-Solvay Division of Allied Chemical and Dye Corporation) found upon analysis to possess the following structural formula:  $C_{143}H_{282}(OH)_6$  and polyisobutylene having a Flory molecular weight of 84,000. The long-chain alcohol wax and the polyisobutylene are employed in the following ratios: 5:0, 4:1, 3:2, 2.5:2.5, 2:3, 30 1:4 and 0:5. The ingredients are heated to a temperature of about 100° C. and mixed with an Eppenbach Homomixer for about one hour until a homogeneous mixture is obtained.

#### EXAMPLE III

35 Another paraffin wax composition in accordance with this invention is obtained by employing as ingredients therefor a paraffin wax having a melting point of 125° F., Alcowax 6 (a product of the Semet-Solvay Division of Allied Chemical and Dye Corporation) found upon analysis to possess the following structural formula:



40 and polyisobutylene having a Flory molecular weight of 587,000. The ingredients are employed in the same percentages and ratios as in Example II and are combined in the same fashion.

#### EXAMPLE IV

45 Still another paraffin wax composition in accordance with the present invention is obtained by employing as ingredients therefor a paraffin wax having a melting point of 125° F., Alcowax G (a product of the Semet-Solvay Division of Allied Chemical and Dye Corporation) found upon analysis to possess the following structural formula:  $C_{131}H_{248}(OH)_{16}$  and polyisobutylene having a Flory molecular weight of about 1,325,000. The ingredients are again employed in the same percentages and ratios as in Example II and are combined in the same fashion.

60

#### EXAMPLE V

55 Yet another paraffin wax composition in accordance with the present invention is obtained by employing as ingredients therefor a paraffin wax having a melting point of 125° F., Alcowax 6 and an isobutylene copolymer made by copolymerizing polyisobutylene and isoprene. About 2 percent of the hydrocarbon present in this copolymer is derived from isoprene, the rest being derived from isobutylene. The Flory molecular weight of the copolymer is 55,000. The ingredients are again employed in the same percentages and ratios as their corresponding ingredients in Example II and are combined in the same fashion.

#### EXAMPLE VI

70 Still another paraffin wax composition in accordance with the present invention is prepared by employing as

ingredients therefor about 99 percent by weight of a paraffin wax having a melting point of 122° F., and a combined total of one percent by weight of Alcowax 6 and polyisobutylene having a Flory molecular weight of 30,000. The long-chain alcohol wax and polyisobutylene are again employed in the same ratios as in Example II and are combined in the same manner.

## EXAMPLE VII

Yet another paraffin wax composition in accordance with the present invention is prepared by employing as ingredients therefor about 90 percent by weight of a paraffin wax having a melting point of 133° F., and a combined total of 10 percent by weight of Alcowax M and polyisobutylene having a Flory molecular weight of 84,000. The long-chain alcohol wax and polyisobutylene are again employed in the same ratios as in Example II and are combined in the same manner.

## EXAMPLE VIII

Another paraffin wax composition in accordance with the present invention is prepared by employing as ingredients therefor about 80 percent by weight of a paraffin wax having a melting point of 130° F. and a combined total of 20 percent by weight of Alcowax 6 and polyisobutylene having a Flory molecular weight of 84,000. The long-chain alcohol wax and polyisobutylene are again employed in the same ratios as in Example II and are combined in the same manner.

## EXAMPLE IX

Yet another paraffin wax composition in accordance with the present invention is prepared by employing as ingredients therefor about 50 percent by weight of a paraffin wax having a melting point of 125° F. and a combined total of 50 percent by weight of Alcowax 7 and polyisobutylene having a Flory molecular weight of 84,000. The long-chain alcohol wax and polyisobutylene are again employed in the same ratios as in Example II and are combined in the same manner.

As noted, I have found that paraffin wax compositions comprising paraffin wax, a rubbery isobutylene polymer and a long-chain alcohol wax, have a higher sealing strength than compositions comprising only paraffin wax and a rubbery isobutylene polymer or paraffin wax and a long-chain alcohol wax, the latter two used within the percentages described above. The compositions containing the three components possess, in addition, superior tensile strength. This is best shown in Tables I and II below wherein the data obtained in testing the paraffin waxes produced in Examples I and II, respectively, are tabulated.

The sealing strength of the paraffin wax compositions was tested in the following manner. A 25-pound sulfite bread wrapper paper was treated with the paraffin wax composition to obtain a uniform deposition of about 12 to 13 pounds of wax composition per ream of 480 24-inch by 36-inch sheets. The waxed paper was then cut into strips 3 inches by 9 inches with the length being parallel to the paper fiber. After the waxed paper strips had been held at a constant temperature of 70° F. for at least 12 hours, they were sealed along the 3-inch width by means of a brass roll heated to a temperature of about 190° and 200° F. and then aged for 24 hours at 70° F. The sealing strength of the seal was then obtained by first trimming the seal to a width of 2 inches and a length of 4 inches, and then determining the amount of tension required to peel the sealed strips apart at a standard rate of pull of 5 millimeters per second. The sealing strength values are reported as grams per linear inch of width. The tensile strength of the paraffin wax compositions was obtained in accordance with TAPPI Tentative Standard T644m-54.

Table I

|   | Paraffin Wax, Percent by Wt. (133 E. M. P.) | Polyisobutylene, Percent by Wt. (84,000 M. W.) | Alcowax 7 | Sealing Strength, Gms./in. | Tensile Strength, Pounds/1/4 in. <sup>2</sup> |
|---|---------------------------------------------|------------------------------------------------|-----------|----------------------------|-----------------------------------------------|
| 5 | 95                                          | ---                                            | 5.0       | 27                         | 198                                           |
|   | 95                                          | 1.0                                            | 4.0       | 33                         | 185                                           |
|   | 95                                          | 2.0                                            | 3.0       | 53                         | 159                                           |
|   | 95                                          | 2.5                                            | 2.5       | 42                         | 156                                           |
|   | 95                                          | 3.0                                            | 2.0       | 55                         | 147                                           |
|   | 95                                          | 4.0                                            | 1.0       | 49                         | 128                                           |
|   | 95                                          | 5.0                                            | ---       | 16                         | 115                                           |

Table II

|    | Paraffin Wax, Percent by Wt. (133 E. M. P.) | Polyisobutylene, Percent by Wt. (84,000 M. W.) | Alcowax M | Sealing Strength, Gms./in. | Tensile Strength, Pounds/1/4 in. <sup>2</sup> |
|----|---------------------------------------------|------------------------------------------------|-----------|----------------------------|-----------------------------------------------|
| 15 | 95                                          | ---                                            | 5.0       | 34                         | 188                                           |
|    | 95                                          | 1.0                                            | 4.0       | 24                         | 168                                           |
|    | 95                                          | 2.0                                            | 3.0       | 31                         | 157                                           |
|    | 95                                          | 2.5                                            | 2.5       | 52                         | 160                                           |
|    | 95                                          | 3.0                                            | 2.0       | 60                         | 133                                           |
|    | 95                                          | 4.0                                            | 1.0       | 60                         | 117                                           |
|    | 95                                          | 5.0                                            | ---       | 16                         | 115                                           |

Data relating to sealing strength obtained from Tables I and II have been employed in the preparation of the curves shown in the accompanying figure, which is hereby incorporated in and made a part of the specification. In the figure, the ratio of the long-chain alcohol wax to polyisobutylene has been plotted against the sealing strengths of paraffin wax compositions containing 133 E. M. P. paraffin wax, polyisobutylene having a Flory molecular weight of 84,000 and Alcowax 7 or Alcowax M. The curve marked 1 refers to the composition containing Alcowax 7, while the curve marked 2 refers to the composition containing Alcowax M. An examination of the curves reveals that paraffin wax compositions containing paraffin wax and selected amounts of a rubbery isobutylene polymer and a long-chain alcohol wax have a higher sealing strength than paraffin wax compositions containing only polyisobutylene or a long-chain alcohol wax. As can be seen, this effect is particularly striking with paraffin wax compositions wherein the weight percent of rubbery isobutylene polymer in the combined total of rubbery isobutylene polymer and long-chain alcohol wax is about 86 to about 52 percent and the weight percent of long-chain alcohol wax is about 14 to about 48 percent.

The data tabulated below further show that paraffin wax compositions comprising paraffin wax, a rubbery isobutylene polymer and a long-chain alcohol wax possess higher sealing strength than compositions containing paraffin wax and only a rubbery isobutylene polymer or a long-chain alcohol wax. The paraffin wax employed in each case had a melting point of 130° F., and the compositions were prepared as in Example II using an Eppenbach Homomixer.

Table III

|    | Paraffin Wax, Percent by Wt. | Polyisobutylene, Percent by Wt. (84,000 M. W.) | Alcowax 6 | Sealing Strength, Gms./in. |
|----|------------------------------|------------------------------------------------|-----------|----------------------------|
| 65 | 97.5                         | 2.5                                            | ---       | 8                          |
|    | 97.5                         | ---                                            | 2.5       | 38                         |
|    | 95.0                         | ---                                            | 5.0       | 26                         |
|    | 95.0                         | 2.5                                            | 2.5       | 74                         |
| 70 | 90.0                         | 5.0                                            | 5.0       | 114                        |

7  
Table IV

| Paraffin Wax, Percent by Wt. | Polyisobutylene, Percent by Wt. (84,000 M. W.) | Alcowax 7 | Sealing Strength, Gms./in. |
|------------------------------|------------------------------------------------|-----------|----------------------------|
| 97.5                         | 2.5                                            | 2.5       | 8                          |
| 97.5                         | ---                                            | 5.0       | 31                         |
| 95.0                         | 2.5                                            | 2.5       | 24                         |
| 95.0                         | 5.0                                            | 5.0       | 40                         |
| 90.0                         | 5.0                                            | 5.0       | 51                         |

Table V

| Paraffin Wax, Percent by Wt. | Polyisobutylene, Percent by Wt. (557,000 M. W.) | Alcowax 7 | Sealing Strength, Gms./in. |
|------------------------------|-------------------------------------------------|-----------|----------------------------|
| 97.5                         | 2.5                                             | 2.5       | 9                          |
| 97.5                         | ---                                             | 5.0       | 31                         |
| 95.0                         | 2.5                                             | 2.5       | 24                         |
| 95.0                         | 1.0                                             | 4.0       | 40                         |
| 90.0                         | 5.0                                             | 5.0       | 53                         |

In each instance in Tables III, IV and V above, compositions containing paraffin wax, a rubbery isobutylene polymer and a long-chain alcohol wax had a higher sealing strength than a paraffin wax composition containing paraffin wax and one only of a rubbery isobutylene polymer or a long-chain alcohol wax. Thus, in Table III a paraffin wax composition containing 95 percent by weight of paraffin wax and 5 percent of Alcowax 6 had a sealing strength of 26 grams per inch, while one containing the same amount of paraffin wax and 2.5 percent of polyisobutylene and 2.5 percent of Alcowax 6 had a sealing strength of 74 grams per inch. When the total weight of Alcowax 6 and polyisobutylene is increased to 10 percent, the ratio between the two remaining the same, the sealing strength was raised to 114 grams per inch. The data in Tables IV and V parallel that of Table III.

In addition to possessing improved sealing strength and tensile strength, the paraffin wax compositions of this invention are also characterized by a superior blocking point. Blocking can be defined as the temperature at which two sheets of paper coated with a wax composition will stick together such that upon separation of the sheets 50 percent or more of the coating is damaged. This is shown in Table VI wherein compositions comprising paraffin wax having a melting point of 130° F., a polyisobutylene having a molecular weight of 84,000 and one of Alcowax M, Alcowax 7, and Alcowax 6 were tested for such property. The compositions were prepared in the manner described in Example I. The blocking point was obtained in accordance with TAPPI Tentative Standard T477m-47.

Table VI

| Paraffin Wax, Percent by Wt. | Polyisobutylene, Percent by Wt. | Alcowax | Blocking Point, °F. |
|------------------------------|---------------------------------|---------|---------------------|
| 95.0                         | 0.5                             | 14.5    | 112                 |
| 95.0                         | 1.0                             | 24.0    | 108                 |
| 95.0                         | 0.5                             | 34.5    | 112                 |

<sup>1</sup> Alcowax M.

<sup>2</sup> Alcowax 7.

<sup>3</sup> Alcowax 6.

The data in Table VI show that representative paraffin wax compositions of this invention have a blocking point of 108° F. or more. This is to be contrasted with the

paraffin wax alone which has a blocking point of but 100° F.

As previously noted, the paraffin wax compositions of this invention are of particular value in coating fibrous materials. The application of the wax compositions to a fibrous base can be performed in any conventional manner and the amount applied thereto will vary with the type of fibrous base and the use to which it is put. In Example X below is shown the application of the paraffin wax compositions of this invention to a paper base.

#### EXAMPLE X

The paraffin wax composition of Example I is placed in a tank and maintained therein as a molten bath at a temperature of about 190° F. The paper to be coated with the paraffin wax composition, a 25-pound white opaque sulfite paper, machine glazed on one side and coated with titanium oxide on the other, is passed successively through the molten wax bath at a linear speed of about 50 feet per minute with an immersion time of one second, a set of squeeze rolls to remove excess wax, and a water bath maintained at a temperature of about 35° F. with an immersion time therein of about one second to chill and solidify the coating on the paper. The coated paper is then wound upon a spool and is ready for use or additional processing. The wax deposition on the paper produced is about 2 grams per square foot of surface area.

In addition to paraffin wax, a rubbery isobutylene polymer and a long-chain alcohol wax, the paraffin wax compositions of the present invention can also contain other additives normally incorporated in paraffin wax compositions for a particular purpose without departing from the spirit and scope thereof. For example, additives such as antioxidants, coloring agents, perfumes, etc., can be added to the paraffin wax compositions without adversely affecting the sealing strength and other properties thereof.

Obviously, many modifications and variations of the invention as hereinabove set forth may be made without departing from the spirit and scope thereof, and therefore only such limitations should be imposed as are indicated in the appended claims.

I claim:

1. An improved paraffin wax composition comprising a major amount of a paraffin wax and a minor amount of a rubbery isobutylene polymer and a long-chain alcohol wax having the following structural formula:



50 wherein  $k$  is an integer from about 50 to about 310 and  $m$  is an integer from one to about 50.

2. An improved paraffin wax composition comprising a major amount of a paraffin wax and a minor amount of a polyisobutylene and a long-chain alcohol wax having the following structural formula:  $C_{k+m}H_{2k+m+2}(OH)_m$ , wherein  $k$  is an integer from about 50 to about 310 and  $m$  is an integer from one to about 50.

3. An improved paraffin wax composition comprising a major amount of a paraffin wax and a minor amount of a rubbery isobutylene polymer and a long-chain alcohol wax having the following structural formula:



65 wherein  $k$  is an integer from about 50 to about 310 and  $m$  is an integer from one to about 50, the weight percent of rubbery isobutylene polymer in said minor amount of rubbery isobutylene polymer and long-chain alcohol wax being about 92 to about 46 percent and the weight percent of long-chain alcohol wax being about 8 to about 54 percent.

4. An improved paraffin wax composition comprising a major amount of a paraffin wax and a minor amount of a polyisobutylene having a Flory molecular weight above about 5,000 and a long-chain alcohol wax having the following structural formula:  $C_{k+m}H_{2k+m+2}(OH)_m$ , where-



and the weight percent of long-chain alcohol wax being about 14 to about 48 percent.

18. A paper having a coating thereon comprising a paraffin wax composition containing at least about 90 percent by weight of a paraffin wax having a melting point of about 133° F. and the remainder polyisobutylene having a Flory molecular weight of about 84,000 and a long-chain alcohol wax having the following structural formula:  $C_{143}H_{282}(OH)_6$ , the weight percent of polyisobutylene in said remainder of polyisobutylene and long-chain alcohol wax being about 86 to about 52 percent and the weight per cent of long-chain alcohol wax being about 14 to about 48 percent.

19. A paper having a coating thereon comprising a paraffin wax composition containing at least about 90 percent by weight of a paraffin wax having a melting point of about 125° F. and the remainder polyisobutylene having a Flory molecular weight of about 587,000 and a long-chain alcohol wax having the following structural formula:  $C_{147}H_{294}(OH)_2$ , the weight percent of polyisobutylene in said remainder of polyisobutylene and long-chain alcohol wax being about 86 to about 52 percent

and the weight percent of long-chain alcohol wax being about 14 to about 48 percent.

20. A paper having a coating thereon comprising a paraffin wax composition containing at least about 90 percent by weight of a paraffin wax having a melting point of about 125° F. and the remainder polyisobutylene having a Flory molecular weight of about 1,325,000 and a long-chain alcohol wax having the following structural formula:  $C_{131}H_{248}(OH)_{16}$ , the weight percent of polyisobutylene in said remainder of polyisobutylene and long-chain alcohol wax being about 86 to about 52 percent and the weight percent of long-chain alcohol wax being about 14 to about 48 percent.

15 References Cited in the file of this patent

UNITED STATES PATENTS

|           |          |       |               |
|-----------|----------|-------|---------------|
| 2,504,400 | Erchak   | ----- | Apr. 18, 1950 |
| 2,698,309 | Thwaites | ----- | Dec. 28, 1954 |
| 2,712,534 | Erchak   | ----- | July 5, 1955  |
| 2,728,735 | Anderson | ----- | Dec. 27, 1955 |